

Nov. 2, 1937.

B. SANFORD

2,097,803

GRINDING WHEEL

Filed Feb. 14, 1935



FIG. 1



FIG. 2

Inventor

BAALIS SANFORD

WITNESSES

Franklin E. Johnson  
WR Greenwood

Clayton H. Jenkins  
Attorney

## UNITED STATES PATENT OFFICE

2,097,803

## GRINDING WHEEL

Baalis Sanford, Worcester, Mass., assignor to  
Norton Company, Worcester, Mass., a corpora-  
tion of Massachusetts

Application February 14, 1935, Serial No. 6,441

2 Claims. (Cl. 51—206)

This invention relates to grinding wheels and more particularly to a composite grinding wheel for use as a cutting-off wheel which has an outer annular grinding portion of diamond grains bonded by an organic bond and an inner central supporting body of a moldable, heat-settable composition and to a method of making the same.

In making a grinding wheel of this type, it has been found that a suitable organic bonding material for the diamond grains is a resinoid material of the heat-settable type, such as a phenolic resinoid of the kind known by the trade-mark of "Bakelite". The usual construction of such wheels comprises a peripheral rim portion composed of diamond grains united by a bond of resinoid and a central supporting body integrally united to the abrasive rim composed of a resinoid molding composition which primarily comprises the bulk of the article. These materials of the respective zones or portions of the wheel may be combined and shaped into a grinding wheel by suitable means and methods. For example, the wheel may be made in accordance with a method which involves "hot pressing" a mixture of diamond grains and resinoid bond in a mold in situ with a preformed resinoid core to form a hard, dense mass and heat setting the resinoid.

It is found, however, that such a method presents certain mechanical difficulties when applied to the manufacture of thin cutting-off wheels, which due to the slender dimensions of the article together with the different coefficients of expansion and unequal shrinkages of the cured materials in the inner and outer zones of the body and the different maturity characteristics possessed by each of the resinoid compositions used, results in a warped final product.

It is accordingly an object of my invention to overcome such difficulties and provide a composite grinding wheel of this type which will not be warped to a detrimental extent after manufacture and which may be economically and easily produced.

It is a further object of my invention to provide a diamond abrasive wheel of a composite structure having a plurality of zones as well as a method of making such an article in which the shrinkages and coefficients of expansion thereof may be made substantially equal, and to provide a wheel structure having substantially uniform shrinkage throughout.

With these and further objects in view, as will be apparent in the following disclosure, my

invention resides in the subject matter described hereinafter and covered by the claims appended hereto.

Referring to the drawing, which illustrates one embodiment of my invention and in which like reference numerals indicate like parts:

Fig. 1 is a plan view of a grinding wheel embodying my invention; and

Fig. 2 is a cross-sectional view, on an enlarged scale, taken on the line 2—2 of Fig. 1.

In accordance with my invention, I propose to make a composite grinding wheel of this type having a peripheral annular abrasive body of resinoid bonded diamond grains and an inner zone or central supporting body of a resinoid composition integrally united therewith, in which there is incorporated suitable granular inert material in such an amount that the relative shrinkages between the inner and outer zones are substantially equalized. That is, the ingredients of the inner and outer zones are so selected and proportioned, and preferably in equal volume percentages in the two zones, that they may be formed into a unitary body of substantially the same structure and shrinkage throughout.

Referring to the drawing, which shows one specific embodiment of my invention, I have there illustrated a grinding wheel having an outer grinding portion or rim 10 of resinoid bonded diamond granules and a center portion 12

of a resinoid composition interspersed with granular inert material. A central hole 13 is provided in the portion 12 for the subsequent mounting of the complete wheel on a spindle. While various resinoid materials may be selected for bonding the diamond grains in the outer rim portion of the wheel and for making the center portion thereof and uniting the granular material incorporated therein, I preferably employ a fusible, potentially reactive, heat-settable resinoid of the phenolic type, such as is commonly known in the art under the trade-mark "Bakelite" and obtained as a condensation product formed by the reaction of phenol and formaldehyde or by that of their homologues. For the granular inert material in the center portion, I may utilize any mineral or non-mineral substances which do not change in size materially under the temperature conditions employed during "hot pressing"; and, for example, I may employ such granular materials as silicon carbide, crystalline alumina or quartz sand.

It is an essential feature of the invention that the volume percentages of bond and grains in the two zones of the wheel shall be sufficiently

alike to prevent a material difference in the shrinkages of the two zones. That is, if the outer zone contains 50% by volume of diamond grains and 50% by volume of bond, then one should use 5 50% by volume of bond and 50% by volume of granular filler in the inner zone. This insures identical shrinkages. Reasonable variations in these proportions are, of course, permissible.

As a specific example of a composition which 10 will be suitable for forming a satisfactory grinding wheel having substantially equal shrinkage throughout, I may utilize the ingredients in the following proportions:

|    |                                      |                   |
|----|--------------------------------------|-------------------|
| 15 | Outer zone                           | Percent by volume |
|    | Diamond grains (100 mesh grit size)  | 50                |
|    | Resinoid bond (phenolic resinoid)    | 50                |
| 20 | Inner zone                           | Percent by volume |
|    | Silicon carbide (100 mesh grit size) | 50                |
|    | Resinoid bond (phenolic resinoid)    | 50                |

It will, of course, be obvious that different grain sizes of the diamonds and the granular filler may be employed and that the various kinds of resinoids may be used accordingly, as is well known in the art. The density and structure of the product are determined by the nature of the ingredients employed as well as their relative proportions. However, it is preferred to form a wheel structure in which the materials of the two portions are compacted into a substantially solid, dense mass, that is, one having practically zero porosity.

The materials of the two portions or zones are mixed separately and in a dry condition until the respective grains of diamond and filler have each been thoroughly incorporated with the particular resinoid bond employed therewith which is in a powdered or finely divided condition. The central support or inner zone of the wheel is first formed by pressure in a cylindrical mold of the size desired for the wheel center which has resulted in a body having compact and reasonably dense structure. Thus, by that method, the dry resinoid mixture as above prepared and incorporating the granular filler is molded by a preliminary compacting operation to produce a strong central support. During this operation, care should be taken to keep the resinoid bond from completely reacting so as not to become converted into the infusible state. This preformed body 12 is then set into a mold cavity of a size to form the complete wheel and an iron core is inserted into the center hole 13 to prevent deformation while under the molding pressure. The dry mixture of diamonds and resinoid is then packed into the mold and pressed in place by a suitable hand implement around the outer periphery of the solid center, after which the whole wheel mass is then subjected to heat and pressure in accordance with the usual "hot pressing" practice which is employed in the art, so that the various sections are molded together and matured into a hard, integral structure of the desired density. Such procedure as that of my prior Patent 1,981,970 may also be used.

It is also feasible to make such a wheel by the following method in which a thin metal ring or annular band is placed in the mold around and spaced from the arbor pin, the diameter and height of this band being the same as the corresponding sizes of the central support in the fin-

ished wheel. The central supporting wheel body is then made by filling the mold space between the ring and the arbor with the resinoid molding composition which includes the inert granular material. The mixture is then tamped in 5 position. Thereafter, the ring is removed from the mold and the remainder of the mold cavity is then filled with the proper amount of diamond and resinoid mixture to make a rim portion 10 of the desired grinding properties. The wheel material is then subjected to heat and pressure whereby the material is molded into an integral unitary body in which the resinoid bond in the two portions is matured and set to its final infusible condition.

It will now be appreciated that this invention applies to a composite wheel structure in which the central non-abrasive portion shrinks either more or less than does the outer diamond rim portion during cooling of the bond in each of the 15 respective portions after it has been matured by heat. If the composition of the central zone contained materials which served to prevent its contracting as much as does the cured diamond and resinoid mixture in the rim, then the greater 20 rim shrinkage would place the center portion under compression and cause warpage or buckling of this center portion. Similarly, if the center portion should shrink more than the outer rim, then either the rim would be placed under radial 25 tension to produce warping of the center, or the two zones might even separate due to the excessive internal strain. Hence, it is desirable in 30 making a multi-zone wheel of this type that the two sections be so constituted that the differential contraction therebetween be equalized, so 35 that when the heated resinoid in each zone of the molded article contracts during cooling, the two zones will act alike and contract equally 40 since they will have the same coefficients of shrinkage. This condition, as above stated, is satisfied by having the resinoid bonds occupy substantially the same volume percentages in the two zones. That is, each bond should occupy 45 the same percentage per unit of volume in each of the zones. For convenience of manufacture, it is also desirable to have the grain size of the diamonds and that of the granular filler in the 50 respective zones of substantially the same size. It is important, however, if strength is to be 55 considered, that the grains of granular inert material in the inner zone be made of a fine grit size, whether or not the diamond grains employed in the rim portion are small in size. Nevertheless, there must be the same total volume of 60 solids per unit of volume in each of the zones. Also, if the resinoids differ in their shrinkage coefficients, then due allowance will be made for this in determining the volume percentages 65 thereof. Hence, the main object of this invention is satisfied by so selecting and proportioning the ingredients that the coefficients of shrinkage of the two zones in the completed article are substantially alike.

Having thus described my invention, what I 65 claim as new and desire to secure by Letters Patent is:

1. A thin cutting off grinding wheel comprising an outer annular abrasive zone of diamond grains and a reacted resinoid bond compacted 70 and proportioned to provide a dense body and a central supporting zone of a granular filler other than diamond and reacted resinoid bond compacted into a rigid support for the outer zone, said granular filler and its bond in the inner 75

zone being so proportioned that the bond occupies substantially the same volume percentage as does the bond of the abrasive zone.

2. A thin cutting off grinding wheel comprising an outer annular abrasive zone of diamond grains and a reacted resinoid bond compacted and proportioned to provide a dense body and a central supporting zone of silicon carbide grains

and reacted resinoid bond compacted into a rigid support for the outer zone, said silicon carbide and its bond being so proportioned that the bond occupies substantially the same volume percentage as does the bond of the abrasive zone and the shrinkages of the two zones are substantially equal. 5

BAALIS SANFORD.